

April 15, 1930.

C. H. ELLIOTT

1,754,745

### ROLLING STRIP METAL

Filed June 13, 1929

3 Sheets-Sheet 1

Fig. 1.



Fig. 2.



INVENTOR  
Charles H. Elliott,  
by his stepson  
Bymer, Bettine Hanley

April 15, 1930.

C. H. ELLIOTT

1,754,745

ROLLING STRIP METAL

Filed June 13, 1929

3 Sheets-Sheet 2



Fig. 3

INVENTOR  
Charles H. Elliott  
Inventor  
Byme, William Runde

April 15, 1930.

C. H. ELLIOTT

1,754,745

ROLLING STRIP METAL

Filed June 13, 1929

3 Sheets-Sheet 3

*Fig. 4.*



INVENTOR

Charles H. Elliott,  
by his attorney,  
Byers, Seltzer & Hanley

## UNITED STATES PATENT OFFICE

CHARLES H. ELLIOTT, OF YOUNGSTOWN, OHIO, ASSIGNOR TO REPUBLIC IRON AND STEEL COMPANY, OF YOUNGSTOWN, OHIO, A CORPORATION OF NEW JERSEY

## ROLLING STRIP METAL

Application filed June 13, 1929. Serial No. 370,685.

This invention relates to the rolling of strip metal, and is of particular value in the rolling of wide thin material.

In the rolling of wide thin strips, such as so-called "strip-sheet," the amount of "crown" or "fullness" of the final product is of importance to the consumer and is also of considerable importance to the manufacturer in that the presence of too much fullness in the material, either as delivered from the last pass of the rolling mill or as delivered from the several passes preceding the final pass, may result in riffling of the product at the edges. If too much riffling occurs, the material is uncommercial and difficulty is encountered in guiding it through the mill. It has heretofore been suggested that in order to satisfactorily roll wide thin material by a continuous process, there should be supplied to the roll train a piece which is convex in cross section, and that the amount of convexity should be progressively reduced in the several stands.

According to the proponents of this system, the factors of roll contour, roll temperature, composition and springiness of the rolls, spacing of the rolls; and shape, composition, and temperature of the piece, must all be taken into account and the successive roll stands so controlled as to provide an active pass in each stand which is less convex than the piece delivered to it from the preceding stand.

According to this system of rolling, it is necessary for highly skilled workmen to watch the several stands of rolls to the end of controlling the variable elements and thus maintaining the desired progressively decreasing convexity in the several stands. It is also suggested by the proponents of this system that furnaces should be placed between the several stands so as to carefully control the temperature of the pieces.

I have found that by using mill stands having backed working rolls, as for example four-high mills, it is possible to eliminate the large amount of skilled labor required in the system above referred to, to eliminate furnaces between mill stands and to successfully roll wide thin material at high speed. In order to at-

tain these results it is necessary to maintain the piece sufficiently flat in the several stands to permit of controlling its direction by side guides. In other words, instead of depending on the convexity of the piece to cause it to track through the stands, I maintain the piece substantially flat in the several stands and use side guides to control it. The backed mills are inherently so stiff that the large roll spring which is characteristic of two-high sheet mills is substantially reduced and it is, therefore, possible to maintain the desired degree of flatness in the piece at all stages. Instead of supplying a convex piece to the backed mills, I supply a piece which is flat or slightly concave. The concavity may be obtained by crowning one of the earlier sets of rolls. I prefer to have the piece slightly concave rather than flat at the beginning of the run, so that it will never become convex, even though the rolls are considerably worn.

Preferably some of the stands are operated as a continuous mill, that is to say, the piece is in two or more passes at one time. During this part of the operation the substantial flatness of the material is particularly valuable because if the metal is properly entered into the continuous stands and is sufficiently flat, no difficulty is encountered in getting it through the mill.

Wide strip material has so much surface area, relative to its mass, that it tends to cool very quickly, particularly in the later stages of the rolling operation. There will, therefore, be encountered a slight spring of the rolls in the later passes, despite the stiffness imparted by the backing rolls. On this account, I prefer that the last pass shall be a relatively light one so as to insure the desired flatness in the final product.

I also prefer to use edging rolls during the earlier stages of the operation. These reduce the tendency to roll full in the center, thus making easier the production of the flat piece which is to be reduced to strip. They also, by the operation of thickening the edges, tend to prevent the more rapid cooling of the edges than the middle, such as ordinarily occurs, and thus they maintain a desirable uniformity

of temperature across the piece during rolling.

In the accompanying drawings illustrating the present preferred embodiment of my invention,

5 Figure 1 is a top plan view, largely diagrammatic, illustrating a rolling mill for carrying out my invention;

Figure 2 is a side elevation thereof;

10 Figure 3 is a diagrammatic view showing the actual contour of pieces rolled in successive stands according to my invention, but with the vertical scale exaggerated; and

15 Figure 4 is a chart showing the limited departure of the piece from true flatness after the several passes.

The mill shown in Figures 1 and 2 comprises heating furnaces 20, from which slabs are supplied to a roll table 21. The slabs pass over a table 22 employing skew rolls to a 20 No. 1 edging pass 23. The edged piece then travels through two two-high stands 1 and 2, then through a No. 2 edger indicated at 24. The piece continues through two-high stands 25 3 and 4 and thence through a No. 3 edger indicated at 25. Beyond this edger there is provided a two-high stand 5, this being followed by four-high stands 6, 7, 8, 9 and 10. The four-high stands employ small work rolls 30 26 and larger backing rolls 27 and are preferably of the type illustrated in the Biggert and Johnson Patent No. 1,654,235. The stands 6 and 7 are grouped together, as shown in Figures 1 and 2, and the stands 8, 9 and 35 10 constitute another group. These last three stands ordinarily operate as a continuous mill, the piece being in all of them at once during a portion of the rolling operation.

40 Roll tables 28 extend between the several stands and support the piece during its travel. The roll tables are provided with side guides as indicated diagrammatically at 29 and in rolling these guides are effective for properly directing the material into the stands and guiding it therethrough. By reason of the fact that the several passes are all substantially flat, the tendency of the rolls to force a sidewise movement of the piece concomitant with its longitudinal travel is 45 eliminated or reduced to the point where such tendency can be easily resisted by the side guides without injuring the strip or causing cobbling. The rolls in the several stands are driven by motors 30, connected through gearing as shown.

50 In the mill above described, I employ flat rolls in stands 1 to 4, inclusive, and use a convex roll in stand 5. The roll is convexed in an amount sufficient to offset the natural roll 55 spring and produce a piece which is flat or slightly concave. While I employ convex rolls in the last two-high stand, it will be understood, of course, that convex rolls might be employed in one of the earlier four-high stands of a given mill to supply a substan-

tially flat piece to the succeeding stands. For that matter, all of the stands might employ backed rolls, but the piece being relatively hotter and thicker in the earlier passes, it will be satisfactory to employ two-high stands 70 for these early passes. However, the later stands should have backed working rolls and care should be taken that in them the material is always maintained sufficiently flat to permit of controlling it by the side guides.

75 The following is a tabulation of the size and character of one set of rolls successfully employed in the manufacture of steel strip 30 inches wide:

Stand No. 1, top working roll  $20\frac{1}{8}$ " diameter; 80 bottom working roll  $20\frac{1}{8}$ " diameter; both rolls flat:

Stand No. 2, top working roll  $21\frac{1}{2}$ " diameter; 85 bottom working roll  $21\frac{1}{2}$ " diameter; both rolls flat:

Stand No. 3, top working roll  $21\frac{3}{4}$ " diameter; 85 bottom working roll  $21\frac{3}{4}$ " diameter; both rolls flat:

Stand No. 4, top working roll  $22$ " diameter; 90 bottom working roll  $21\frac{1}{8}$ " diameter; both rolls flat:

Stand No. 5, top working roll  $22\frac{3}{4}$ " maximum diameter, crown .028 inches in diameter; bottom working roll  $22\frac{1}{8}$ " diameter, flat. Total width of crown on top roll is 95  $15\frac{1}{2}$ " on each side of the center line of the roll,  $6\frac{1}{2}$ " to either side of the center line of the roll being flat:

Stand No. 6, top working roll  $15\frac{1}{4}$ " diameter; 100 bottom working roll  $15\frac{1}{4}$ " diameter; both rolls flat:

Stand No. 7, top working roll  $15\frac{7}{8}$ " diameter; 105 bottom working roll  $15\frac{3}{4}$ " diameter; both rolls flat:

Stand No. 8, top working roll  $16\frac{3}{4}$ " diameter; 105 bottom working roll  $16\frac{1}{8}$ " diameter; both rolls flat:

Stand No. 9, top working roll  $16\frac{5}{8}$ " diameter; 110 bottom working roll  $16\frac{1}{2}$ " diameter; both rolls flat:

Stand No. 10, top working roll  $16\frac{1}{2}$ " diameter; 115 bottom working roll  $16\frac{7}{8}$ " diameter; both rolls flat:

The diameter of the backing rolls, in each of the stands 6 to 10, inclusive, was  $32$ ". All 115 rolls had bodies  $42$ " long.

The analysis of the steel being rolled was as follows:

|            | Per cent |
|------------|----------|
| Carbon     | .08      |
| Manganese  | .39      |
| Phosphorus | .012     |
| Sulphur    | .029     |

The slabs used were  $30\frac{1}{2}$ " x  $2\frac{1}{2}$ " x  $58$ " and were successively reduced in stands 1 to 5, inclusive, so that the material when it issued from stand No. 5 had a thickness on the center line of  $.327$ ", and by reason of the crowning of the top roll in this stand showed a concavity at the center of approximately  $.003$ ". 130

Figure 3 shows lines 5 to 10<sup>o</sup>, inclusive, illustrating the contour of the piece after leaving each of the passes 5 to 10, inclusive.

The curves of Figure 3 were obtained by measuring the thickness of the piece at substantially half inch intervals across its entire width and plotting the readings thus obtained. It will be understood that in this view the vertical scale has been greatly exaggerated so as to show the variations in thickness or contour.

The following is a tabulation of the thickness at the center line:

|                           |       |
|---------------------------|-------|
| After leaving No. 5 pass  | .327" |
| After leaving No. 6 pass  | .241" |
| After leaving No. 7 pass  | .151" |
| After leaving No. 8 pass  | .111" |
| After leaving No. 9 pass  | .085" |
| After leaving No. 10 pass | .070" |

It will be noted that the material is substantially flat after each of the passes, there being a slight thinning at the edges but the body portion of the sheet being very flat.

Figure 4 illustrates in chart form the departure from true flatness after the several passes. In this chart the line D<sup>1</sup> illustrates the convexity or concavity of the piece after each pass from stand No. 5 on. It will be noted that at stand 5 there is .003" concavity and that from stands 6 to 8, inclusive, there is .004" convexity. At stand 9 the convexity has increased to .0065" and then drops off again to .005" in the last pass.

Considering the convexity of the body portion of the sheet, that is to say, disregarding the slight thinning of the edges, and considering only that portion of the sheet lying between the lines L<sup>1</sup> and L<sup>2</sup> of Figure 3 (the lines L<sup>1</sup> and L<sup>2</sup> lying three inches inwardly from the edges), the departure of the material from true flatness is illustrated in Figure 4 by the line D<sup>2</sup>. This line shows that over the main body portion of the sheet there is a concavity of .002" when the material enters the first four-high stand and that thereafter there is a convexity ranging from .0005" to .0015". This remarkable flatness of the material is highly desirable in the finished product and makes it possible to control the material by side guides during its passage through the mill.

So far as I am aware, my invention is applicable to the rolling of thin material of any width. It eliminates any necessity for heating furnaces between the stands and beyond the usual amount of supervision does not require highly skilled employees. Neither does it require the close calculation of roll contour required in other systems, since the inherent stiffness of the backed mill makes it possible to use flat rolls in many passes. It is to be understood that the rolls may be turned to other than flat profile, depending on the particular conditions encountered, so long as

there is produced in different stands a piece of sufficient flatness to permit of controlling it by side guides.

I have illustrated and described a present preferred embodiment of the invention. It will be understood, however, that it is not limited to the form shown, but may be otherwise embodied and practiced within the scope of the following claims.

I claim:

1. In the method of rolling strip metal in backed mills, the steps consisting in passing material through successive roll stands, engaging its edges between stands to guide it and maintaining it sufficiently flat in the several passes to permit of controlling it by side guides.

2. In the method of rolling strip metal in backed mills, the steps consisting in supplying a concave piece, passing it through successive roll stands, engaging its edges between stands to guide it and maintaining it sufficiently flat in the several passes to permit of controlling its direction by side guides.

3. In the method of rolling strip metal in backed mills, the steps consisting in passing material through successive roll stands, engaging its edges between stands to guide it, maintaining it sufficiently flat in the several passes to permit of controlling it by side guides, and taking a relatively light draft in the final pass.

4. In the method of rolling strip metal in backed mills, the steps consisting in supplying a piece substantially without convexity in cross section, passing it through successive roll stands, engaging its edges between stands to guide it and maintaining it sufficiently flat in the several passes to permit of controlling it by side guides.

5. In the method of rolling strip metal in backed mills, the steps consisting in passing material through successive roll stands, engaging its edges between stands to guide it, maintaining it sufficiently flat in the several passes to permit of controlling it by side guides and engaging it during a portion of the rolling operation in a plurality of stands at one time.

6. In the method of rolling strip metal, the steps consisting in subjecting a heated piece to reducing and edging passes so as to produce a piece substantially free of convexity in cross section, and rolling it in backed mills.

7. In the method of rolling strip metal, the steps consisting in subjecting a heated piece to reducing and edging passes so as to produce a piece substantially free of convexity in cross section, rolling it in backed mills, and maintaining the piece sufficiently flat in the several backed mill passes to permit of controlling it by side guides.

In testimony whereof I have hereunto set my hand.

CHARLES H. ELLIOTT.